

## UNITED STATES PATENT OFFICE

2,244,093

## ROOFING AND THE LIKE

Richard A. Wilkins, Rome, N. Y., assignor to  
 Revere Copper and Brass Incorporated, Rome,  
 N. Y., a corporation of Maryland

No Drawing. Application March 4, 1941,  
 Serial No. 381,697

2 Claims. (Cl. 108—13)

My invention relates to roofing and the like, and particularly to improvements in the roofing forming the subject matter of my pending application Serial Number 363,515, filed October 30, 1940.

As pointed out in the above mentioned pending application, the material heretofore commonly employed for copper roofing, sheathing, and other exposed protective coverings for buildings has been thin rolled sheets of highly refined copper. Further, in refining copper for these purposes it has heretofore always been the practice of producers thereof to remove so far as possible all impurities so as to secure as pure a copper as possible. The known high resistance of pure copper generally to chemical corrosion, and the observed fact that impurities commonly found in rolled copper tend to make it less ductile in both the hot and cold rolled conditions, more difficult to produce by either hot or cold rolling, and commonly "cold short" in the sense that it tends to crack when bent or otherwise cold worked, have caused pure copper heretofore to be considered the most satisfactory commercially available material for light weight metal roofing and the like. In fact during the past forty years copper roofing has for these reasons been made almost exclusively of electrolytically refined copper, which commonly is 99.9% pure copper.

Nevertheless it is a frequently observed fact that copper roofing, even when substantially 100% pure electrolytically refined copper, often fails in use, being subject to cracking sufficient to render it non-waterproof. Heretofore it was believed that these cracks were caused by mechanical fatigue resulting by reason of the cyclic stresses set up by alternate expansion and contraction of the copper sheets under varying temperature conditions. For that reason builders heretofore have resorted to expensive roof constructions, and various expensive expedients such as corrugating the roofing and the employment of elaborately designed expansion joints, and the use of heavy gauge copper in the attempt to relieve or reduce the effect on the roofing of these cyclic stresses and thereby eliminate so far as possible this form of failure. Although these attempts have been partially successful, the expense incidental thereto, and the many failures which actually have occurred in spite of these precautions, have seriously interfered with the general adoption of this otherwise very satisfactory roofing.

As pointed out in applicant's pending appli-

cation above referred to, applicant has found that the failure of copper roofing and the like heretofore has not been correctly understood. This material, he has found, does not fail primarily by reason of the cyclic stresses to which it is subjected when in use, as heretofore believed, but, strangely enough, primarily by reason of a heretofore wholly unsuspected type of corrosion which occurs when this highly pure copper is exposed to an atmosphere contaminated by wind borne products of combustion of modern domestic and industrial fuel burning appliances and industrial atmospheres in general.

Applicant has found, that upon removing the patina and other accumulated corrosion products from copper roofing which has failed, the copper roofing surface thus exposed is characteristically pitted, instead of being in its smooth unpitted condition in which it originally left the rolling mill or the metal showing a uniform decrease in thickness over its whole surface due to corrosion.

His investigations show that these pits are caused by the formation on the copper, when exposed to a contaminated atmosphere, of a film of corrosion products which is characterized by a lack of adhesion to the copper, a lack of tenacity in respect to failure, and a tendency toward perviousness which allow the copper to be attacked locally rather than uniformly by the corrosive media and thereby result in the formation of sharply defined, inwardly pointed pits in the nature of notches. He has found that copper so attacked rapidly fails when subjected to the cyclic stresses hereinbefore referred to by reason of the natural tendency of the stresses to be concentrated in the metal below the bottoms of the notch-like pits. As a result of this concentration of the stresses, the metal below the bottoms of the pits "work hardens" and the fatigue strength of the material is exceeded, and as a result the metal cracks at the pits.

Pure copper roofing applicant has found is comparatively sensitive to this "notch effect," when caused by a combination of chemical corrosion and subjection to cyclic stresses, on account of the film which forms on it causing the pure copper to pit and the great sensitivity of pure copper to work hardening when cold worked.

The above mentioned application points out that this type of failure of copper roofing as constructed from thin sheets, commonly from 0.003 to 0.03 inch in thickness, can be substan-

tially entirely avoided by incorporating into the copper controlled amounts of arsenic.

When arsenic is incorporated it has been found that the surface of the copper, after the patina or other accumulated products of corrosion are removed, is in an unpitted condition, any corrosion which has occurred being substantially uniformly distributed over its surface. Also it has been found that the arsenic most markedly decreases the sensitivity of the copper to work hardening when cold worked, and therefore any scratches, dents, or the like in the nature of notches which might be formed during the handling or installation of the roofing will not cause it to fail by notch effect. In other words, the action of the arsenic is twofold: it prevents notches from being formed by corrosion and prevents the roofing failing by notch effect even if the notches are accidentally formed by mechanical means.

It has been found that the presence of the proper amount of arsenic in the copper roofing produces on the roofing surface a corrosion film which is tenacious, adherent, impervious and non-hygrosopic, the film being comparably as ductile as the copper base material itself, thus permitting the roofing to be repeatedly bent without rupture of the film or interruption of its adherence to the copper. Thus this film effectively protects the underlying base material from contaminated air and moisture, and in this way effectively eliminates the possibility of the formation of the above mentioned notch-like pits, for any slight amount of corrosion which occurs will be uniformly distributed over the surface of the copper. Most importantly this film has the property of being self-healing in the sense that if for any reason its continuity is locally interrupted it will substantially immediately reform when subjected to corrosion and thus act to prevent substantial local corrosion at the interrupted regions which in a pure copper would continue to corrode at an accelerated rate resulting in pitting at the point of interruption of the film.

The above mentioned application points out that the beneficial effects of arsenic in copper roofing are obtained with additions of 0.02 to 1.5% arsenic, the maximum beneficial effects being secured with about 0.05%. Applicant has now found that, in place of adding arsenic to the copper, the same and improved beneficial effects may be secured by adding controlled amounts of antimony.

Antimony, it has been found, causes the formation on the exposed copper roofing surface, of a corrosion film, consisting predominantly of antimony content compound, having substantially the same physical and chemical properties as the hereinbefore described film which forms when arsenic is added to the copper, this film caused by the addition of antimony forming substantially immediately when the copper roofing surface is exposed to contaminated air, moisture, or other corrosive media, and being self-healing in the same sense as the film formed when arsenic is added. It further, like arsenic, reduces the sensitivity of the copper roofing to work hardening, and because of this and because it causes the formation of the above mentioned film antimony, like arsenic, substantially prevents the possibility of failure of the roofing by notch effect. Antimony, however, to a much greater degree than arsenic secures a marked increase in the tensile strength of the copper

5 roofing, commonly about a 15 to 20% increase, and as it is desirable to have the roofing strong as well as resistant to notch effect, and as antimony is a less expensive metal than arsenic and commonly more easily obtained commercially, it forms a desirable substitute for arsenic.

Appreciable effects will be secured with as little as 0.05% antimony. The beneficial effects increase with an increase in the antimony up to 10 about 0.8%, above which value the antimony tends to cause the copper to become cold short in the sense that cold working either during fabrication or when subjected to cyclic stresses after installation tends to form therein minute 15 surface cracks analogous to notches. When "de-oxidized" copper is employed, the antimony exists in the copper-antimony alloy in solid solution with the copper. With copper containing oxygen it exists in the copper-antimony alloy 20 for the most part in the form of a secondary phase which apparently consists of copper, antimony and oxygen, the remainder being in solid solution with the copper. The effect of the antimony in either case however is the same in 25 respect to the properties hereinbefore mentioned, and for this reason the much less expensive copper containing oxygen is preferably employed.

When adding antimony best results ordinarily 30 will be secured when the roofing does not contain impurities which tend to render it less malleable in the hot and cold conditions and thus tend to cause the hot or cold rolling or other working of the roofing during its fabrication to result in sub-microscopic surface cracks therein analogous in 35 their effects to pits.

Among these deleterious substances are lead, 40 bismuth, iron, nickel and sulphur, very small amounts of all of which tend to make the copper roofing more difficult to produce, and all of which tend to make the antimony bearing copper roofing approach the poor resistance of pure copper roofing to corrosion and its sensitivity to notch effect, and thereby act to destroy the beneficial effects of the antimony. The presence of such 45 substances as cobalt, tin, silicon and zinc in substantial amounts had also best be avoided as they tend to increase the sensitivity of the copper roofing to work hardening and notch effect. Thus it will be understood, that in the sense the copper roofing does not contain deleterious substances or amounts thereof which substantially destroy the beneficial effects tended to be imparted by the antimony, the balance of the alloy aside from the antimony is essentially copper.

In making the roofing according to the invention the copper may be melted, and the antimony added to the melt in the form of a copper-antimony alloy rich in antimony. The molten metal may then be cast into slabs, which latter may be rolled into sheets of desired thickness by the usual mill process of rolling copper roofing sheets. Finally the rolled sheets are annealed to the degree of softness that will best resist the cyclic stresses to which they are subjected when in use.

For convenience in terminology the article of manufacture according to the invention is termed "roofing," it being understood that as used in the appended claims such term includes various shingles, sheetings, valleys, and like protective coverings for buildings, as well as what in a more limited sense is ordinarily termed "roofing." Also it will be understood that the roofing according to the invention comprises sheet copper presenting an extensive external roofing surface, and may in this sense consist of a backing

having an exterior sheet of copper as well as consist wholly of sheet copper.

I claim:

1. Roofing comprising sheet copper presenting an extensive external roofing surface, the copper being alloyed with such amount of antimony between 0.05 and 0.8% as will cause the formation on said surface when exposed to atmospheric corrosion of a self-healing, adherent, protective film composed predominantly of antimony content compound, while rendering the sheet copper

less sensitive to failure by reason of notch effect than sheet copper without the antimony when subjected to the cyclic stresses caused by expansion and contraction of the roofing.

5 2. Roofing comprising sheet copper presenting an extensive external roofing surface, the copper being alloyed with approximately 0.05 to 0.8% antimony, the balance of the alloy in respect to the antimony being essentially copper.

RICHARD A. WILKINS.